

May 5, 1936.

E. O. RHODES

2,039,450

METHOD OF TREATING ROAD SURFACES

Filed April 10, 1931

PARTICLES OF SOLID  
BITUMINOUS MATTER  
SHORTLY AFTER APPLICATION.



Fig: 1

THICKENED BINDER FORMED  
AFTER APPLIED PARTICLES  
HAVE FLUXED WITH ORIGINAL  
BINDER



Fig: 2

INVENTOR.  
Edmund O. Rhodes.

BY  
Jesse R. Langley, ATTORNEY.

## UNITED STATES PATENT OFFICE

2,039,450

## METHOD OF TREATING ROAD SURFACES

Edmund O. Rhodes, Pittsburgh, Pa., assignor to  
American Tar Products Co., Inc., a corporation  
of Delaware

Application April 10, 1931, Serial No. 529,068

7 Claims. (Cl. 94—23)

This invention relates to a method of treating road surfaces, particularly of the types which are laid cold and are known as bituminous macadam or bituminous concrete roads.

5 An object of the present invention is to provide a method whereby an improved road surface may be secured and it may be rendered impervious to air and moisture.

A further object is to provide a method where-  
10 by a previously laid bituminous macadam or bi-  
tuminous concrete road may be treated to im-  
prove the bituminous binder in the road mix-  
ture.

It is customary to construct roads with a pre-  
15 mixed material composed of the desired grade  
of mineral aggregate and a bituminous binder.  
Ordinarily the binder would have a float test at  
32° C. of 100 to 300 seconds (A. S. T. M. method  
D139-27). The premixed material is placed upon  
20 the road and rolled to produce a relatively smooth  
surface. To render the surface less pervious to  
air and moisture, it has been the practice to ap-  
ply thereto a sealing coat of hot tar or asphalt  
after the premixed material has "set up."

25 The present process comprises spreading on the  
surface of a road prepared from material con-  
taining mineral aggregate and a bituminous bind-  
er, particles of a bituminous substance which is  
adapted to coalesce with the binder. The mix-  
30 ture of mineral aggregate, such as crushed stone,  
and bituminous binder, such as tar or asphalt,  
are put in place in the usual manner and then  
rolled. A powdered or granular bituminous ma-  
35 terial is then preferably immediately distributed  
over the surface of the road. The powdered bi-  
tuminous material may be mixed with a filler, if  
desired.

Any of the well known bituminous materials  
40 which may be readily ground into a powder or into  
granular form may be used, as, for example,  
pitches from coal tars or oil tars, Trinidad, Ber-  
mudez, Cuban or petroleum asphalts and even  
bituminous substances, such as those mentioned,  
45 containing dispersions of coal. In other words,  
any bituminous material which is hard enough to  
be ground to produce particles of from 8 to 20  
mesh down to an impalpable powder may be  
used. Materials are used having a cube-in-air  
50 melting point of 115—160° C. when tested in the  
apparatus described in Fischer Scientific Co.'s  
(Pittsburgh, Pa.) Catalogue under the number  
1-665 and in J. Ind. Eng. Chem. 10 817, (1918).

The best results are obtained by the use of a  
bituminous material having a low temperature  
55 susceptibility in the range of temperatures en-

countered in nature and which when spread on  
the road surface, will coalesce with the binder  
and thereby increase the viscosity and melting  
point thereof.

Examples of filler which may be used with the  
5 powdered bituminous material are rock dusts,  
stone screenings, hydrated lime, sand, celite and  
lampblack. These fillers may be mixed with the  
bituminous powders in any desired proportions,  
as, for instance, equal parts of each.

The amount of powdered bituminous materials  
distributed on the surface of a road depends upon  
the texture thereof and the more porous the sur-  
face, the greater the quantity required to seal it.  
Ordinarily 2 to 6 pounds of powdered bituminous  
10 material per square yard of road surface may be  
used. The particles may be brushed into the sur-  
face or after they have been uniformly distributed  
they may be rolled.

In the accompanying drawing, Figures 1 and 2  
20 are sectional views of a pavement shown in two  
different stages.

In both figures a layer of a mixture of aggre-  
gate 1 and binder 2 with voids 3 is shown on a  
road bed 4.

25 In Fig. 1, particles of pitch 5 are shown dis-  
tributed over the surface of the layer in such a  
manner that at least the pits and crevices formed  
by the spaces between the pieces of stone are  
filled. Of course the pitch may be applied to form  
30 a layer of any desired depth.

By treating a road surface in the manner de-  
scribed above, the hard pulverized bituminous  
material, upon coming in contact with a soft  
35 binder 2 already present in the road surface mix-  
ture, fluxes with the soft binder as shown at 6  
and increases the hardness thereof. In the draw-  
ing, the distances between the stones are some-  
what exaggerated to more clearly indicate the  
change which takes place.

40 Besides obtaining a moisture and air impervious  
layer, the road surface is made tougher and more  
resistant to deformation. A quicker "set up" of  
the road surface is brought about than by the  
natural agencies of evaporation, oxidation and  
45 polymerization.

I claim as my invention:

1. A method of preparing a road surface which  
comprises forming a surface layer containing bi-  
50 tuminous binder material of relatively low sta-  
bility and then spreading on the said surface  
layer solid particles consisting of solid material  
substantially entirely bituminous, adapted to co-  
alesce substantially entirely with, and to increase  
55 the stability of, said surface layer in its upper

portion by mixing with the said binder material in said portion of said layer.

2. A method of preparing a road surface which comprises spreading on a road bed a road material comprising bituminous material of relatively low stability to form a layer and then spreading on the surface of the said layer solid particles consisting of solid material substantially entirely bituminous, of relatively high viscosity and 5 adapted to coalesce with the bituminous material of said layer by mixing therewith in the upper portion of the said layer to thereby materially increase its stability in such upper portion.

3. A method of preparing a road surface which 15 comprises providing a layer of road material consisting at least in part of relatively soft binder which material is of relatively low stability, and spreading on the said layer of road material comminuted pitch of relatively high viscosity and 20 melting point and which is adapted to coalesce and mix with said binder in the upper part of the said layer to thereby produce a combined bituminous mixture the viscosity and the melting point of which are materially higher than 25 those of said binder, the said mixture forming a seal for said road surface.

4. A method of treating a surface of a road constructed of materials including a layer of mineral aggregate and a bituminous binder, 30 which method comprises distributing on the sur-

face of the said layer solid particles consisting of solid material substantially entirely bituminous and having a melting point of 115° C. to 160° C., and subjecting the said layer to pressure and a distributing action to bring about coalescence of the said solid particles with the said binder in the upper stratum of the said layer and to thereby form a seal for the surface of said layer. 5

5. A method of preparing a road surface which 10 comprises mixing aggregate and a bituminous binder of relatively low viscosity, spreading the mixture, and subsequently distributing on the surface of the spread mixture finely divided hard bitumen and finely divided filler. 15

6. A method of preparing a road surface which comprises mixing aggregate and a bituminous binder of relatively low viscosity, spreading the mixture, and subsequently distributing on the 20 surface of the spread mixture finely divided hard bitumen and finely divided filler in substantially equal parts by weight per square yard of road surface.

7. A method of preparing a road surface, which 25 comprises mixing aggregate and a bituminous binder of relatively low viscosity, spreading the mixture, and subsequently distributing on the surface of the spread mixture hard bitumen particles.

EDMUND O. RHODES. 30